

May 3, 1960

A. DUNBAR ET AL

2,934,885

PROCESS FOR ARMORING CABLE

Filed Aug. 13, 1957



**FIG. 2 -**



**FIG. 4 -**



**FIG. 3 -**



INVENTORS.  
Alver Dunbar, George J. Hausmann  
& Bayard S. Johnson,  
BY Paul & Paul  
ATTORNEYS

1

2,934,885

## PROCESS FOR ARMORING CABLE

Alver Dunbar, Philadelphia, Pa., George J. Hausmann, Merchantville, N.J., and Bayard S. Johnson, Ardmore, Pa., assignors to Franklin Research Company, Philadelphia, Pa., a corporation of Pennsylvania

Application August 13, 1957, Serial No. 678,009

7 Claims. (Cl. 57—162)

This invention relates to improvements in armoring cable, and more particularly relates to a process for armoring cable with strands coated with bituminous or asphalt material or the like and preventing the coated strands from sticking.

In the armoring of cables with strands of metal covered with a coating of asphalt-coal tar or the like, it is the usual practice to pass twenty-four of such coated strands to an armoring machine where the strands are twisted together in a spiral fashion about a cable. In this manufacture the coated strands become hot and sticky because of friction as the strands contact the guides and sheaves of the armoring machine. This causes peeling or stripping of the coating and gumming up of the guides and sheaves and forces a stoppage of the armoring machine for a difficult cleaning operation. It has long been a problem to overcome such stickiness and to eliminate troubles caused thereby in the armoring machine. As far as is known, however, previous attempts to solve this problem have not proved entirely successful.

Accordingly, an object of this invention is to overcome the aforementioned defects. Another object is to armor cable with bituminous coated metal strands and prevent undesirable sticking of one strand to another and to other objects during the process.

Another object is to armor cable with bituminous coated strands more quickly and more efficiently than has previously been accomplished. Another object is to keep the armoring machine running for longer periods of time without cleaning than has heretofore been possible.

Other objects and advantages of this invention will further become apparent hereinafter and in the drawings in which:

Fig. 1 represents a view in side elevation and partly diagrammatic of apparatus constructed for practicing the present invention;

Fig. 2 represents an enlarged sectional view taken as indicated by the lines and arrows II—II which appear in Fig. 1;

Fig. 3 represents an enlarged sectional view taken as indicated by the lines and arrows III—III which appear in Fig. 1; and

Fig. 4 represents a diagrammatic view of apparatus for practicing this invention.

Although specific terms are used for clarity in the following description, these terms are intended to refer only to the structure shown in the drawings and are not intended to define or limit the scope of the invention.

Turning now to the specific embodiment of the invention selected for illustration in the drawings, the number 11 designates generally an adhesive coating machine (Fig. 4), and the numbers 12 and 13 designate respectively a non-adhesive coating machine and an armoring machine. An armor wire 14 which is preferably of high tensile steel and which is covered with a cotton braid sheath is impregnated with hot asphalt-coal

2

tar in the adhesive coating machine 11. This operation provides armor wire 14 with a bituminous or asphalt coating 15. If desired, the cotton braid sheath is omitted and the bituminous coating is applied directly to armor wire 14.

Then bituminous coated armor wire 14 is passed to non-adhesive coating machine 12 where it is provided with a non-adhesive coating 16. After this, wire 14 is dried and is wound on spools.

10 To armor a cable, a plurality, usually twenty-four, of spools of armor wire 14 with coatings 15 and 16 are passed to an armoring machine 13. Here each coated armor wire 14 is operated upon by guides and sheaves and the wires 14 are twisted about a coaxial cable in a spiral fashion to armor the cable. After this, the armored cable is given a coating of asphalt-coal tar.

Turning to the non-adhesive coating machine 12 shown in Fig. 1, machine 12 is provided with a tank 18 which contains a liquid 21 which is brought into tank 18 through pipe 22. Also provided is an overflow pipe 23.

20 Positioned in tank 18 is a wheel 24 which is rotatable about a horizontal axis 25 and has formed in its perimeter a groove 26. Mounted above wheel 24 is a brush 27 having bristles 28. Brush 27 and bristles 28 are so positioned that bituminous coated wire 14 passes between the brush and the groove 26 as is shown in Fig. 2. Wheel 24 has its lower portion submerged in liquid 21 and the rotation of wheel 24 brings liquid 21 into contact with bristles 28 and with coating 15 of wire 14 to form a film of the liquid 21 on coating 15. This film of liquid 21 forms coating 16.

25 In the practice of the present invention, the composition of the anti-adhesive material used in forming coating 16 is important. Therefore, preferred examples of suitable anti-adhesive composition for use in the practice of the present invention are set forth below.

## Example 1

|    | A. Wax emulsion:                  | Parts by wt. |
|----|-----------------------------------|--------------|
| 40 | Refined paraffin                  | 793          |
|    | Starch                            | 35½          |
|    | Caustic soda                      | 21           |
|    | Duponol SO (sodium octyl sulfate) | 13¾          |
|    | Water                             | 2982         |

## 45 B. Metallic salt:

Basic aluminum acetate,  $\text{Al}(\text{C}_2\text{H}_3\text{O}_2)_2\text{OH}$  186

The basic aluminum acetate of B was dissolved in a part of the water content listed for the wax emulsion 50 A and then added with stirring to the wax emulsion of A.

## Example 2

Zinc acetate and zirconium acetate, respectively, were 55 used in place of the basic aluminum acetate of Example 1, in each case in the amount of 186 parts by weight dissolved in a portion of the water content listed for the wax emulsion A of Example 1.

## Example 3

|    | A. Wax emulsion:                                                                | Parts by wt. |
|----|---------------------------------------------------------------------------------|--------------|
| 60 | Refined paraffin                                                                | 600          |
|    | Starch                                                                          | 50           |
|    | Alrosperse 11P (fatty amine condensate) (Alrose Chemical Co.)                   | 12           |
| 65 | Neutronyx 600 (100% active aromatic polyglycol ether) (Onyx Oil & Chemical Co.) | 12           |
|    | Atlas G-3920 (polyoxyethylene oleyl ether)                                      | 12           |
|    | Water                                                                           | 2720         |

70 B. Metallic salt:

|                                                                                |     |
|--------------------------------------------------------------------------------|-----|
| Basic aluminum acetate, $\text{Al}(\text{C}_2\text{H}_3\text{O}_2)_2\text{OH}$ | 372 |
|--------------------------------------------------------------------------------|-----|

## Example 4

| A. Wax emulsion:                              | Parts by wt. |
|-----------------------------------------------|--------------|
| Refined paraffin                              | 180          |
| Oxidized microcrystalline paraffin (Crown 36) | 20           |
| Emulsifier                                    | 40           |
| Water                                         | 720          |
|                                               | 960          |

  

| B. Metallic salt:                           |     |
|---------------------------------------------|-----|
| Basic aluminum acetate, $Al(C_2H_3O_2)_2OH$ | 240 |

One part by weight of the metallic salt of B dissolved in a small portion of the water of A was mixed with 4 parts by weight of the wax emulsion of A. The emulsifier for the refined paraffin was non-ionic consisting of a mixture in equal parts of polyoxyethylene oleyl ether (Atlas G-3920) and the monostearate of sorbitan (Span 60). Both products are made and sold by Atlas Powder Co. of Wilmington, Delaware.

## Example 5

| A. Wax emulsion:                                         | Parts by wt. |
|----------------------------------------------------------|--------------|
| Ouricury wax                                             | 289.5        |
| Refined paraffin                                         | 144.5        |
| Polyethylene glycol monostearate (molecular weight 1000) | 102          |
| Tween 40 (sorbitan monopalmitate)                        | 25.2         |
| Formaldehyde                                             | 20           |
| Water                                                    | 1494         |

  

| B. Metallic salt:                           | Percent solution |
|---------------------------------------------|------------------|
| Basic aluminum acetate, $Al(C_2H_3O_2)_2OH$ | 28               |

One part by weight of a 28% solution of basic aluminum acetate is mixed with four parts by weight of the wax emulsion of A although it should be noted that aluminum acetate solution is miscible with the emulsion of A in all proportions. The resulting composition provides a film which dries with a gloss which is advantageous under certain conditions of use.

The composition of the anti-adhesive material used in the practice of the present invention consists broadly of a liquid containing a water soluble waxy material or an emulsified water insoluble material and the component which on drying will form a water resistant film containing a metallic salt of an acid selected from the group consisting of hydrochloric acid, hydrobromic acid, formic acid and acetic acid, with the metal being selected from the group consisting of aluminum, zinc and zirconium.

The waxy film and metallic salt thus deposited form in the pores and on the surface of coating 16 as either the hydroxide or the oxide of the metal salt. It has been discovered that such an oxide or hydroxide waxy film has the peculiar and unexpected property of resisting the normal adhesion which occurs between wires 14 with coating 15.

In the above examples it should be noted that carnauba wax, sugar cane wax, or equivalent synthetic waxes may be used in conjunction with the refined paraffin or in place thereof.

It has been found in the practice of this invention that undesirable sticking has been eliminated in armoring machines to such an extent that the production of the armoring machine has been increased by 25 percent. On unwinding the spools of armor wire, non-adhesive coating 16 helps to prevent stripping or peeling of the braid as the armor wire comes off the spool. Coating 16 also helps prevent gumming up of the guides and the sheaves in the armoring machine. Previously, shutting down the armoring machine would cause the armor wire braid and its bituminous coating to stick to the guides and sheaves. On subsequent starting of the armoring machine, this

sticking would cause the cotton braid to pull or peel from wire 14. Now, with the use of coating 16, this does not happen. Very little of the coatings 15, 16 are transferred from wire 14 to the guides and sheaves of the armoring machine. Further, coating 16 acts as a lubricant in the armoring operation.

Having thus described our invention, we claim:

1. A process of armoring a cable comprising the steps of applying a coating of bituminous material to a strand; applying to the outer surface of said bituminous material a film comprising an aqueous solution of a salt of a metal selected from the group consisting of aluminum, zinc and zirconium, in combination with a binder comprising a waxy material; drying said film to an adherent non-adhesive condition; and twisting the strand together with similar strands about a cable.

2. A process of armoring a cable comprising the steps of applying a coating of bituminous material to a strand; applying to the outer surface of said bituminous material a film comprising an aqueous solution of a metallic acetate selected from the group consisting of aluminum acetate, zinc acetate and zirconium acetate, in combination with a binder comprising a waxy material; drying said film to an adherent non-adhesive condition; and twisting the strand together with similar strands about a cable.

3. A process of armoring a cable comprising the steps of applying a coating of bituminous material to a strand; applying to the outer surface of said material a film comprising an aqueous solution of a metallic salt of an acid selected from the group consisting of hydrochloric acid, hydrobromic acid, formic acid and acetic acid, with the metal being selected from the group consisting of aluminum, zinc and zirconium, in combination with a binder comprising a waxy material; drying said film to an adherent non-adhesive condition; and twisting the strand together with similar strands about a cable.

4. A process of armoring a cable comprising the steps of applying a coating of asphalt-coal tar to a strand; applying to the outer surface of said tar a film comprising an aqueous solution of a metallic salt of an acid selected from the group consisting of hydrochloric acid, hydrobromic acid, formic acid and acetic acid, with the metal being selected from the group consisting of aluminum, zinc and zirconium, in combination with a binder comprising a waxy material; drying said film to an adherent non-adhesive condition; and twisting the strand together with similar strands about a cable.

5. In the process of armoring a cable with a plurality of strands covered with an asphalt material, the method of coating the outer asphalt surface of each of said strands with a film comprising an aqueous solution of a metallic acetate selected from the group consisting of aluminum acetate, zinc acetate and zirconium acetate, in combination with a binder comprising a waxy material.

6. In the process of armoring a cable with a plurality of strands covered with an asphalt material, the method of coating the outer asphalt surface of each of said strands with a film comprising an aqueous solution of a salt of a metal selected from a group consisting of aluminum, zinc and zirconium, in combination with a binder comprising a waxy material.

7. In the process of armoring a cable with a plurality of strands covered with an asphalt material, the method of coating the outer asphalt surface of each of said strands with a film comprising an aqueous solution of a metallic salt of an acid selected from the group consisting of hydrochloric acid, hydrobromic acid, formic acid and acetic acid, with the metal being selected from the group consisting of aluminum, zinc and zirconium, in combination with a binder comprising a waxy material.

## References Cited in the file of this patent

| UNITED STATES PATENTS |                    |               |
|-----------------------|--------------------|---------------|
| 1,420,911             | Davis et al. ----- | June 27, 1922 |
| 2,124,993             | Youmans -----      | July 26, 1938 |
| 2,155,403             | Cook -----         | Apr. 25, 1939 |
| 2,248,123             | Sackner -----      | July 8, 1941  |

|                        |                |
|------------------------|----------------|
| Thiel -----            | Sept. 2, 1941  |
| Thiel -----            | Dec. 30, 1941  |
| Powell -----           | Sept. 16, 1947 |
| Angiolino et al. ----- | Sept. 29, 1953 |
| Owens -----            | July 15, 1958  |